

## UNITED STATES PATENT OFFICE

2,053,151

## CEMENTED TANTALUM CARBIDE

Floyd C. Kelley, Schenectady, N. Y., assignor to  
General Electric Company, a corporation of  
New York

No Drawing. Application October 28, 1930,  
Serial No. 491,814

10 Claims. (Cl. 75—136)

- The present application is a continuation-in-part of my copending application, Serial No. 478,557, filed August 28, 1930, and relates to hard, tough metal compositions generally known as cemented carbides. A composition of this general character is disclosed in Schröter Reissue Patent No. 17,624 and consists of a carbide of an element of the sixth group of Mendelejeff's table of elements of the periodic system, for example tungsten carbide, with a metal of the iron group, for example cobalt, the latter acting as a cementing or binder medium for tungsten carbide particles in the composition.
- Cemented carbide produced in accordance with the process disclosed in the above Schröter patent is somewhat difficult to shape or grind and special grinding wheels, for example carborundum wheels, are usually employed for this purpose.
- It is one of the objects of the present invention to provide a hard, tough, cemented carbide tool which may be shaped or ground easily and supplied with a keen cutting edge by means of ordinary grinding wheels. It is a further object to provide a cemented carbide tool suitable for cutting steel. Other objects of the invention appear hereinafter.

In carrying out my invention, I employ tantalum carbide as the main constituent of the cemented carbide, the binder or cementing medium consisting of two metals, one an element of the sixth group of Mendelejeff's table of elements and the other a metal of the iron group. The tantalum carbide may be prepared by adding about 12 grams of carbon, for example gas coke, to 181.5 grams of tantalum, and milling the tantalum and carbon together for about five hours. The milling produces a very intimate mixture of the materials which are then fired at a temperature varying from 1550 to 1600° C. for about 8 hours in a closed graphite tube and in a hydrogen furnace. A similar carburizing process is disclosed in my copending application, Serial No. 308,565, filed September 26, 1928.

The carbide thus formed is golden brown in color and is milled to break it up into a fine powder capable of passing through a 250 mesh screen. It is then mixed with a suitable amount of a metal binder medium, for example with about 13% of a mixture of iron and molybdenum, the iron and molybdenum being present in the binder preferably in the ratio of about 63 parts by weight of iron to about 37 parts of molybdenum. The mixture of tantalum carbide and

binder material is pressed into any desired shape in a hydraulic press.

The pressed material, usually in the form of a tool bit, is sintered in a closed graphite tube in a hydrogen furnace at a temperature of about 1400° C. for about 1½ hours. If the cemented tantalum carbide bit thus formed is copper brazed to a steel shank, it is desirable to employ a flux, for example borax, in order to secure a good joint.

Cemented tantalum carbide having the above composition has a hardness of about 87.8 on the Rockwell A scale and a modulus of rupture of about 86,750 pounds per square inch, the latter figure being obtained on a tool bit as fired and without previous lapping.

Special grinding wheels, such as carborundum wheels, are not required to shape the cemented tantalum carbide, since it may be shaped easily and quickly by grinding on an ordinary emery wheel. The cemented carbide may be given a very keen cutting edge which it is able to retain under severe operating conditions.

Although the cemented tantalum carbide composition containing about 13% binder material has a relatively low modulus of rupture as compared with that of cemented tungsten carbide employing the same quantity of binder material, a tool bit of this composition gives very satisfactory results. For example, a tool bit constructed as above described when tested on a nickel steel log with a cut of  $\frac{3}{8}$ ", a feed of 55 mils for 10 minutes at 70 feet per minute was perfectly sharp at the end of the test and showed no signs of wear at any point. The same tool without being resharpened was again tested for 8 minutes at 90 feet per minute with the same cut and feed and then for 11 minutes at 100 feet per minute with the same cut and feed as before. The tool maintained its sharp cutting edge and showed very little wear.

Ordinarily, in the use of cemented carbide lathe cutting tools, there is a tendency for the metal chip to wear a slight depression just back of the cutting edge of the tools. I have found however, that this difficulty is avoided when cemented tantalum carbide tool bits are employed. Cemented tantalum carbide tool bits also have the ability to take unusually fine finishing cuts on either steel or cast iron at relatively high speeds. On steel for example, I have taken cuts  $\frac{1}{8}$ " deep with  $1/64$ " feed at speeds as high as 300 feet per minute. The finish obtained under such conditions is similar to that obtained by

the use of a grinding wheel. It is my present opinion that the ability of cemented tantalum carbide to produce a smooth finish and to remove the material from the work without injury to the tool bit, is due to the fact that the cemented tantalum carbide apparently cuts the metal and does not drag it off.

As a binder material for tantalum carbide, I prefer to employ the eutectic composition consisting of about 63 parts iron and 37 parts molybdenum and having a melting point of about 1440° C. My invention however is not limited to this particular binder. Other binder or cementing mediums may be employed with tantalum carbide if desired, for example a binder consisting of an iron-molybdenum compound constituting of about 53 parts molybdenum with about 47 parts iron and having a melting point of about 1530° C., or a binder consisting of about 45 parts nickel and about 55 parts tungsten and having a melting point of 1460° C., or a binder consisting of about 66 parts nickel and about 34 parts tungsten and having a melting point of 1495° C. However, I have obtained the most satisfactory results with molybdenum-iron binders and particularly with the eutectic binder consisting of about 63% iron and about 37% molybdenum.

Although I have described my invention in connection with a composition consisting of 87% tantalum carbide and 13% binder material, the invention is not limited to these particular percentages. The above quantities, while illustrative of my invention may be varied considerably depending upon the qualities desired in the finished material.

What I claim as new and desire to secure by Letters Patent of the United States, is:

1. A sintered, hard, metal composition consisting of tantalum carbide and a binder medium therefor, said binder medium comprising about 3 to about 20% of said composition and consisting substantially of about 34% to about 55% of metal of the sixth group of Mendelejeff's table of elements of the periodic system and about 45% to about 66% of metal of the iron group.
2. A sintered, hard, metal composition consisting of tantalum carbide and a binder medium therefor, said binder medium comprising about 3 to about 20% of said composition and consist-

ing substantially of about 34% tungsten and 66% nickel.

3. A sintered, hard, metal composition consisting of tantalum carbide and a binder medium therefor, said binder medium comprising about 3 to about 20% of said composition and consisting substantially of about 63 parts by weight of iron and 37 parts by weight of molybdenum.

4. A sintered, hard, metal composition consisting of tantalum carbide and a binder medium therefor, said binder medium comprising about 3 to about 20% of said composition and consisting substantially of about 53 parts by weight of molybdenum and about 47 parts by weight of iron.

5. A hard, tough, cemented carbide composition containing from about 3 to about 20% of a binder material, the remainder of the composition being tantalum carbide, said binder containing about 45 parts by weight nickel and about 55 parts by weight of tungsten.

6. An alloy comprising substantially 9% by weight of molybdenum, substantially 11% by weight of nickel, and substantially 80% by weight of tantalum carbide.

7. An alloy comprising substantially 9% by weight of tungsten, substantially 11% by weight of nickel, and substantially 80% by weight of tantalum carbide.

8. A sintered composition consisting substantially of tantalum carbide particles, metal of the iron group and metal of the sixth group of Mendelejeff's periodic table of elements, said tantalum carbide particles being bonded into a hard, tough mass by a cementing medium consisting substantially of said metal of the iron group and said metal of the sixth group.

9. An alloy consisting substantially of tantalum carbide, metal of the iron group and metal from a group consisting of tungsten and molybdenum, the tantalum carbide comprising at least 80% by weight of said alloy.

10. An alloy consisting substantially of tantalum carbide, nickel, and metal from a group consisting of tungsten and molybdenum, the tantalum carbide comprising at least 80% by weight of said alloy and the nickel being in excess of the metal from said group.

FLOYD C. KELLEY. 50